

C. H. CHANDLER,  
LEAD PLATING,  
APPLICATION FILED MAR. 21, 1918.

1,322,408.

Patented Nov. 18, 1919.

*Fig. 1.*



*Fig. 2.*



*Inventor:*  
Charles H. Chandler

*by* *Ans Spauld.*  
*attorney*

# UNITED STATES PATENT OFFICE.

CHARLES HALLSTRAM CHANDLER, OF NEWPORT, RHODE ISLAND.

## LEAD-PLATING.

1,322,408.

Specification of Letters Patent. Patented Nov. 18, 1919.

Application filed March 21, 1918. Serial No. 223,817.

To all whom it may concern:

Be it known that I, CHARLES H. CHANDLER, a citizen of the United States, residing at Newport, county of Newport, State of Rhode Island, have invented certain new and useful Improvements in Lead-Plating, of which the following is a specification.

This invention relates to lead plating and particularly to the electro-deposition of a lead coating on steel, iron or other vessels or objects subject in their usage to rust or corrosion.

As illustrative of the practice of my invention I shall discuss the lead plating of torpedo air flasks as a specific instance of great immediacy of practical importance.

In plating such an object as a torpedo air flask it is of great importance that the lining be a smooth tough non-corrodible skin so perfectly united to the flask wall that it will not be ruptured or dislodged by expansion or contraction of the vessel either by changes of pressure or temperature.

Furthermore, it is of great practical importance to be able to line large vessels or coat other extensive surfaces rapidly and at a minimum of labor and expense.

In accordance with my invention I am able to deposit electrolytically a hard homogeneous coating of lead very rapidly and economically.

In practising my invention I preferably make an electrolyte by building up a solution of lead carbonate or white lead in hydrofluosilicic acid with a small amount of gelatin or glue. The electrolyte should contain at least 8% of lead and the free acid should be under 5%. These percentages may vary slightly but it is to be noted that 40 should the lead fall below 5% a dark slimy deposit is formed. The gelatin should be added to about 1 per cent. with which the lead deposits in a smooth and solid coating of specific gravity 11.40, the tensile strength 45 being considerably greater than lead in its ordinary form.

In the accompanying drawings, I have illustrated apparatus for the practice of my invention.

50 Figure 1 is a transverse section of a torpedo air flask that is being coated according to my method, and

Fig. 2 is a partial longitudinal section thereof.

55 In practising my invention the air flask

with one head ground on is entirely freed on its inner surface from grease or foreign matter and filled with the electrolyte 2, in any suitable manner.

The flask is connected preferably at several points so as to form the cathode. The electrical connections are indicated at 3.

The anode 4 for such a flask is preferably prepared by casting, in a cylindrical or other convenient form. This may be of pure lead or may be of some suitable alloy if a coating other than of pure lead is desired.

The anode should be supported out of contact with the flask and should be immersed in the electrolyte and is suitably connected in the circuit, as indicated at 5. The feed wires 3 and 5 are connected with the respective poles of any suitable electric energizer (not shown).

With a pure lead anode as described and with an electrolyte containing 10.5% lead and 3½% free acid, I have been able to deposit lead coatings, indicated generally at 6, at the rate of 3.847 grams per ampere hour or 4.9 ampere days per pound. The current density being from 12 to 20 amperes per square foot of surface.

The casting of the lead anodes is a very inexpensive and convenient form of preparing the anode and supplying the lead. The qualities of lead transported by current are comparatively large so that only a relatively small amount of power is necessary, the lead having very favorable physical and electrochemical constant for deposition.

Lead coatings deposited in this manner cover the steel completely and are most tenacious, being only removable by digging off with a sharp instrument. It resists severe treatment such as brushing with a steel brush, and the coating remains smooth and uniform through considerable degrees of expansion and contraction of the flask, and is a most effective preventive against the usual 100 corrosive effects.

My invention as set forth is capable of a variety of modifications and a variety of usages, all without departing from the spirit and such modifications are to be construed as within my invention if within the limits defined by the appended claims.

What I therefore claim and desire to secure by Letters Patent is:

1. The method of lining a torpedo flask

or the like, consisting in gradually electrolytically depositing on it as a cathode a thin dense leaden coating internally thereof from an electrolyte from a lead salt of hydrofluosilicic acid contained within the flask.

2. The method of lining a torpedo flask or the like, consisting in filling said flask shell with an electrolyte containing a lead salt of hydrofluosilicic acid in the proportions of substantially 8% lead and hydrofluosilicic acid not exceeding 5% free, connecting said flask shell as a cathode and in suspending in said contained electrode and out of contact with said flask shell a lead anode and in passing a current therethrough.

3. The method of coating a metallic body, consisting in gradually electrolytically depositing on it as a cathode a dense leaden

skin from an electrolyte consisting of a lead salt of hydrofluosilicic acid. 20

4. The process of depositing a lead coating on the surface of a metal object consisting in forming an electrolyte containing a lead salt of hydrofluosilicic acid having substantially 8% lead and less than 5% free 25 acid and substantially .1% gelatin, and in exposing a leaden anode and the surface to be coated in said electrolyte in anode and cathode relation.

In testimony whereof I affix my signature in presence of two witnesses.

CHARLES HALLSTRAM CHANDLER.

Witnesses:

EDWARD O. RIGGS,  
ELMER BERT COTTRELL.